# EUROPEAN PATENT SPECIFICATION

(11) **EP 1 229 168 B1**
(45) Date of publication and mention of the grant of the patent: **25.04.2007**
(21) Application number: 01102333.0
(22) Date of filing: 01.02.2001
(51) Int. Cl.: E01C 5/00

(54) **Road surface and method for its construction**
Strassendecke und Verfahren zu ihrer Herstellung
Revêtement routier et son procédé de construction

(43) Date of publication of application: 07.08.2002
(73) Proprietor: Albrecht Braun GmbH, 73340 Amstetten (DE); Maer S.p.A., 12048 Sommariva Bosco (Cuneo) (IT); Starka Betongindustrier, 24722 Södra Sandby (SE); Weissenböck Baustoffwerk Gesellschaft m.b.H, 2620 Neunkirchen (AT); Spedalso Betonvarefabrik AS, 8700 Horsens (DK)
(72) Inventor: Ghia, Vittorio, 12040 Sommariva Perno, Cuneo (IT); Braun, Albrecht, Dipl.-Kfm., Albrecht Braun GmbH, 73340 Amstetten (DE); Persson, Lars H., 245 63 Hjärvp (SE); Weissenböck, Karl, Mag., 2620 Neunkirchen (AT); Voldby, Eric E., 8766 Nr. Snede (DK)
(74) Representative: Popp, Eugen

(56) References cited:
- EP-A- 0 456 035
- GB-A- 395 288

## Description

The invention relates to a surface for roads used by vehicular traffic, comprising a road pavement which is supported by a roadbed and comprises prefabricated paving stones made of natural or artificial materials, in particular concrete paving stones, that are laid on a bituminous sand bed, as well as a method for the construction of such a road surface.

The known coverings designed to strengthen roads used by vehicular traffic, in addition to uninterrupted surfaces made of material that becomes hard, such as concrete or asphalt, also include surfaces made of paving stones, in particular concrete paving stones. Surfaces of the latter type have proved useful in particular for courtyards, the entrances to petrol stations, streets where traffic is restricted and the like. The advantage is that when individual stones become damaged, the roadway can be fully repaired merely by replacing these particular stones. Furthermore, when work on the roadbed is to be carried out it can be accessed without problem and, when the work is completed, the road surface can be restored to its original state. Because there are gaps between the individual paving stones, which are usually filled with sand, it is characteristic of such road surfaces that they allow rain and melted snow to flow directly into the ground below, which is desirable in many cases and makes stone pavements particularly valuable from the viewpoint of protecting the environment. However, there is an associated risk that the soil will become contaminated by harmful fluids or solid materials, which can be carried into the ground by the flowing water. For this reason it is problematic to build the roadbed for stone pavements out of demolition products, which are very often contaminated.

Accordingly, the object of the present invention is to provide a construction that is substantially watertight, but nevertheless preserves the advantages of stone paving as cited above.

This object is achieved by the characterizing features of Claim 1, insofar as the road surface itself is concerned, and by those of Claim 10 with regard to the method for construction of such a road surface.

A sand bed with a bitumen component amounting to between 1.5% and 2.5% by weight behaves similarly to a conventional sand bed containing no binding agents at all; that is, even after the bed has been laid and the paving stones vibrated into place, with a corresponding compaction of the sand bed, the latter retains its free-flowing property and does not form solid clumps. Despite this characteristic, the bituminous sand bed provides a layer that is nearly impermeable to water. It should be kept in mind here that the water permeability of a conventional asphalt surface is about 20 to 25%. In contrast, the sand bed in accordance with the invention has a water permeability of maximally 6 to 7%. In comparison with an asphalt surface, therefore, the road surface with a sand bed in accordance with the invention is practically impermeable to water. If the bitumen component amounts to less than 1.5% by weight, the water permeability increases appreciably. On the other hand, with a bitumen component of more than 2.5% by weight there is a risk that the individual sand grains will stick together, in particular after they have been warmed by prolonged insolation. Furthermore, while the sun is shining on the surface a sand bed with a relatively high proportion of bitumen is in danger of "softening", with the consequence that when it is exposed to fairly large forces, in particular a stream of traffic, it will become deformed and make the road surface uneven. This danger exists especially when some of the traffic passing over the road surface consists of heavy goods vehicles.

That contamination of the soil by percolating water that passes through the gaps in a paving-stone surface can be a problem has of course been recognized before. To solve this problem, EP 0 456 035 A2 proposes that clay minerals should be added to the sand in the roadbed, for example montmorillonite and mineral aggregates, in a proportion of up to about 30%. The aim is to produce a sand bed that is relatively watertight. To achieve a sufficiently dense consistency, the proportion of clay minerals and mineral aggregates must be relatively high, with the consequence that the sand-bed mixture is correspondingly expensive. Furthermore, experiments have shown that the water-impermeability of such a sand bed corresponds at most to that of a conventional asphalt road surface.

DE-AS 1 093 396 describes a method of laying down pavement with bituminously bound sand that is characterized by the use of a known binding agent with at least two components, one of which is a powdery, bituminous material and the other an oily, high-boiling-point liquid capable of dissolving the bituminous material. This method is likewise distinguished by the relatively large effort and expense required to construct the sand bed, and the method is designed not to produce a sand bed that is substantially watertight but rather to allow the paving stones to be more firmly embedded in the sand bed, so that it is no longer necessary to fill the gaps between adjacent paving stones. For this purpose the mixture described above is preferably supplemented with adhesive agents such as hydrated lime powder. This adhesive agent is intended to promote fixation of the pavement in the sand bed. The oily additive serves to preserve the mobility or fluidity of the sand components.

The object of the method proposed in DE-AS 1 093 396 thus has nothing to do with the construction of a largely watertight sand bed and correspondingly watertight road surface.

The method in accordance with the invention is distinguished by the fact that on top of a roadbed, which can even be made of demolition products, a sand bed is constructed that in addition to raw sand contains bitumen in a proportion of between 1.5 and 2.5% by weight. Subsequently paving stones are laid down on this sand bed, in such a way that there are gaps between adjacent stones. Prior to the laying of the paving stones the sand bed has not yet been compacted. After laying, the paving stones are vibrated or hammered into the sand bed described here in such a way that bituminous sand rises into the gaps between adjacent stones. At the end of this process the sand bed has become sufficiently compacted, by about 10 to 20%. Because of this compaction, and owing to the bitumen component, the sand bed becomes largely watertight while retaining a flexibility similar to that of a conventional sand bed.

After the paving stones have become fixed within the sand bed, the gaps between them can be filled with conventional jointing sand, which where necessary can also be bituminized. In a preferred embodiment for road construction the sand bed is spread out with a thickness of about 3.0 to 5.0 cm. In the region of the paving stones the sand bed becomes compacted by about 0.5 to 1.0 cm.

Furthermore, experience has shown that when the sand has the preferred granulation and grain-size distribution, as specified in Claim 2, during fixation of the paving stones in the sand bed by vibration or hammering the sand of the bed rises into the gaps between adjacent paving stones by about 0.3 to 0.6 cm, given a gap width of about 0.2 to 0.5 cm. As a result, the paving stones are sufficiently stabilized in the horizontal direction, i.e. in the direction parallel to the road surface, with no need for filling the gaps.

With regard to a preferred sand composition and to preferred compositions of the bitumen component, reference is made to Claims 2, 5, 7, 8.

In the following, preferred exemplary embodiments are described in detail with reference to the attached drawing. This shows a road surface on a roadbed 1, which can comprise demolition products; the road surface comprises a sand bed 2 and, laid thereon, concrete paving stones 3. The concrete paving stones are laid in such a way that between adjacent stones there are gaps 4 with a width of 0.2 to 0.5 cm. In the illustrated embodiment the gaps 4 have been filled from above with jointing sand 5. After the paving stones 3 are placed on the originally uncompacted sand bed 2, the paving stones 3 are vibrated or hammered into the sand bed 2 by means of a surface vibrator 6. The action of the vibrator 6 causes the sand bed in the region of the paving stones 3 to become condensed by at least about 10 to 20%, in particular about 15%. That is, a sand bed with an initial thickness or height of about 3 to 5 cm is compacted in the region of the paving stones so that its thickness or height becomes about 0.5 to 1.0 cm smaller than the initial thickness or height. During this compaction process displaced sand flows from below into the gaps 4 between adjacent paving stones 3 and ascends within these gaps, by about 0.5 cm when the gap width is 0.2 to 0.5 cm.

Experiments have shown that compaction of the sand bed is particularly great in the region of the edges of the paving stones that lie within the sand. That is, the sand of the sand bed 2 is particularly strongly compacted in the region of the gaps; as a result, in combination with the presence of a bitumen component in accordance with the invention and the quality and grain-size distribution of the sand, which are described below, the sand bed is particularly watertight in this region. Surprisingly, with a sand bed in accordance with the invention a water permeability of maximally 6.0 to 7.0% can be achieved, whereas the water permeability of a conventional asphalt surface is up to 25%.

In order further to increase the degree of water impermeability in the joint region, the gaps 4 between adjacent paving stones 3 can additionally be filled from above with jointing sand, in particular bituminous jointing sand.

It is especially advantageous for the weight of the bitumen component of the sand bed 2 to amount to between about 1.8 and 2.2% of the total weight of the sand bed.

Furthermore according to the invention, the distribution of coarse and fine grains in the sand bed 2 is chosen to be such that the action of a surface vibrator 6 on paving stones 3 laid on the originally uncompacted sand bed causes the sand to become compacted by about 10 to 20%, in particular about 15%.

The grain-size distribution of the sand bed 2 for a maximal grain size of 2.0 to 4.0 mm, in particular about 3.0 mm, and for a minimal grain size of about 0.05 to 0.1 mm, in particular about 0.07 to 0.1 mm, is as follows:
Ca. 0-5% of the grains are smaller than 0.10 mm
Ca. 0-15% of the grains are smaller than 0.15 mm
Ca. 5-30% of the grains are smaller than 0.30 mm
Ca. 30-55% of the grains are smaller than 0.50 mm
Ca. 55-80% of the grains are smaller than 1.00 mm
Ca. 80-95% of the grains are smaller than 2.00 mm
Ca. 95-100% of the grains are smaller than 3.00 mm
Ca. 100% of the grains are smaller than 4.00 mm

Expressed somewhat more generally, the grain-size distribution chosen for the sand bed 2 is such that the grain size increases approximately as follows:
In the fine-grain region: linearly to progressively
In the intermediate region: approximately linearly
In the coarse-grain region: regressively

As mentioned above, the gaps 4 between adjacent paving stones can be filled from above with jointing sand 5, in which the proportion of finest grains (grain size ≤ 0.10 mm) is about twice as large as that in the sand bed 2. The grain size of the jointing sand preferably increases slightly progressively throughout.

Another factor of significance for the low water permeability of the road surface from 0.01 to 6.0% and in particular from 0.10 to 3.50%, is the quality of the bitumen for the sand bed 2. The bitumen used here preferably has a density of 1.0 to 1.06 g/cm³ at 25°C, a paraffin component of about 2.0 to' 2.5% by weight, a needle penetration at 25°C of about 60 to 200 dmm (= 1/10 mm), a ductility at 25°C of about 90 to 100 cm, and a viscosity at 135°C of about 200 to 250 mm²/s. Bitumen of this quality permanently encloses the sand grains in such a way that they cannot adhere to one another and form clumps. Sand to which such bitumen has been added remains substantially as free-flowing as raw sand, even after it has been compacted as described above by vibration of the paving stones.

Preferably as the starting material for the sand bed a crushed sand is used, with a grain-size distribution such that the empty-space content of a dry-compacted sample is maximally about 37.0 to 39.0, in particular about 38.5% by volume.

The construction of a road surface with paving stones laid on a sand bed 2 of the kind described here has been described in detail above. Here reference is explicitly made to that description.

Regarding the grain-size distribution for the jointing sand used to fill the gaps, it should be mentioned that this is preferably as follows:
Ca. 0 to 15% of the grains are smaller than 0.07 mm
Ca. 10 to 15% of the grains are smaller than 0.15 mm
Ca. 20 to 30% of the grains are smaller than 0.30 mm
Ca. 35 to 60% of the grains are smaller than 0.6 mm
Ca. 50 to 75% of the grains are smaller than 1.00 mm
Ca. 70 to 90% of the grains are smaller than 2.00 mm
Ca. 85 to 100% of the grains are smaller than 3.00 mm
Ca. 100% of the grains are smaller than 4.00 mm

Intra-plant experiments have shown that the water permeability of a sand bed with an original thickness or height of about 4 cm, with grain sizes and distribution as given in Claim 3, and in which the bitumen component amounted to about 2.0% by weight, was on average about 0.05%. This slight water permeability, in comparison to conventional asphalt or tar surfaces, is practically equivalent to 100% watertightness, so that the road surface in accordance with the invention is considerably better suited for covering contaminated roadbeds than conventional road surfaces made of asphalt or tar. The impermeability of the road surface described here is almost the same as that of concrete. However, the road surface described here offers the great advantage over concrete, as well as over an asphalt or tar surface, that an opening made in the surface can be closed again with no difficulty, so that the original quality of the road surface is preserved. In particular it is surprising that the flexibility of the bituminated sand corresponds closely to that of dry raw sand, even when the road surface described here has been in use for a long time and/or is continuously in use.

In the gap region the compaction of the sand bed is somewhat higher than in the region below the paving stones.

### List of reference numerals

- 1: Roadbed
- 2: Sand bed
- 3: Concrete paving stones
- 4: Gaps
- 5: Jointing sand
- 6: Surface vibrator

## Claims

1. Road surface for areas used by vehicular traffic, comprising a pavement which is supported by a roadbed (1) and which comprises prefabricated paving stones (3) made of natural or artificial materials, in particular concrete paving stones, that are laid on a bituminous sand bed (2),
wherein the bitumen component of the sand bed (2) with respect to the overall weight of the latter amounts to between about 1.5% to 2.5%, by weight, in particular about 1.8% to 2.2% by weight,
**characterized in that:**
the distribution of coarse and fine grains in the sand bed (2) is such that under the action of a vibrator on paving stones (3) laid on the originally uncompacted sand bed, the sand is being compacted by about 10 to 20%, in particular about 15%.

2. Road surface according to Claim 1, **characterized in that** the grain-size distribution of the sand bed (2) for a maximal grain size of 2.0 to 4.0 mm, in particular about 3.0 mm, and for a minimal grain size of about 0.05 to 0.10 mm, in particular about 0.07 to 0.01 mm, is as follows:
Ca. 0 to 5% of the grains are smaller than 0.10 mm
Ca. 0 to 15% of the grains are smaller than 0.15 mm
Ca. 5 to 30% of the grains are smaller than 0.30 mm
Ca. 30 to 55% of the grains are smaller than 0.50 mm
Ca. 55 to 80% of the grains are smaller than 1.00 mm
Ca. 80 to 95% of the grains are smaller than 2.00 mm
Ca. 95 to 100% of the grains are smaller than 3.00 mm
Ca. 100% of the grains are smaller than 4.00 mm.

3. Road surface according to one of the claims 1 or 2, **characterized in that** the paving stones (3) on the sand bed (2) are laid in such a way that they are separated by gaps (4) and are kept apart from one another by sand that rises into the gaps (4) from below.

4. Road surface according to Claim 3, **characterized in that** the gaps (4) between adjacent paving stones (3) are filled from above with jointing sand (5), in which the proportion of the finest grains with grain size ≤0.10 mm is about twice as large as that in the sand bed (2).

5. Road surface according to one of the claims 1 to 4, **characterized in that** the grain size increases approximately as follows:
Sand bed:
In the fine-grain region: linearly to progressively, in the intermediate region: approximately linearly, in the coarse-grain region: regressively
Jointing sand:
Progressively increasing throughout the range.

6. Road surface according to one of the claims 1 to 5, **characterized in that** it has a water permeability of maximally between 0.01 and 6.00%, in particular 0.10 to 3.50%.

7. Road surface according to one of the claims 1 to 6, **characterized in that** the bitumen for the sand bed (2) has a density of about 1.0 to 1.06 g/cm³ at 25°C, a paraffin component of about 2.0 to 2.5% by weight, a needle penetration at 25°C of about 60 to 200 dmm, a ductility at 25°C of about 90 to 100 cm, and a viscosity at 135°C of about 200 to 250 mm2/s.

8. Road surface according to one of the claims 1 to 7, **characterized in that** for the sand bed (2) a crushed sand is used with a grain-size distribution such that the proportion of empty space within a dry-compacted sample is maximally about 37.0 to 39.0, in particular about 38.5% by volume.

9. Road surface according to one of the claims 1 to 8, **characterized in that** the roadbed (1) beneath the sand bed (2) is constructed of demolition products.

10. Method for the construction of a road surface with paving stones (3) laid on a sand bed (2), in particular a road surface according to one of claims 1 to 9, **characterized by** the following steps:
a. the erection on a roadbed (1) of an overlying sand bed (2) containing bitumen in a proportion of 1.8% to 2.2% by weight;
b. the placement of paving stones on the still uncompacted sand bed, so as to leave gaps between adjacent paving stones;
c. the vibration or the hammering of the paving stones into the sand bed in such a way that bituminized sand ascends into the gaps between adjacent paving stones, the distribution of coarse and fine grains in the sand bed being such that during said vibration or hammering the sand bed is compacted by about 10 to 20%, in particular about 15%.

11. Method according to Claim 10, **characterized in that** when the paving stones are vibrated or hammered into the sand bed, bituminized sand ascends into the gaps between adjacent paving stones by a distance of about 0.3 to 0.6 cm, given a gap width of about 0.2 to 0.5 cm.

12. Method according to one of the claims 10-11, **characterized in that** the sand bed is spread out in a thickness of about 3.0 to 5.0 cm.

13. Method according to one of the claims 10-12, **characterized in that** after the paving stones have become fixed within the sand bed, the gaps between adjacent paving stones are filled with jointing sand, in particular bituminized jointing sand.

## Patentansprüche

1. Straßenbelag für Bereiche, die von Kraftfahrzeugverkehr genutzt werden, eine Pflasterung umfassend, die von einer Bettung (1) getragen ist, und die vorgefertigte Pflastersteine (3) aus natürlichem oder künstlichem Material, insbesondere Betonpflastersteine umfasst, die auf einem Bitumen-Sandbett (2) verlegt sind,
wobei der Asphaltbestandteil des Sandbetts (2) im Hinblick auf das Gesamtgewicht des Letztgenannten zwischen ca. 1,5 bis 2,5 Gew.-%, insbesondere ca. 1,8 bis 2,2 Gew.-% beträgt,
**dadurch gekennzeichnet, dass**:
die Verteilung grober und feiner Körner im Sandbett (2) dergestalt ist, dass unter der Einwirkung eines Rüttlers auf die Pflastersteine (3), die auf dem ursprünglich unverdichteten Sandbett verlegt wurden, der Sand um ca. 10 bis 20%, insbesondere um ca. 15% verdichtet wird.

2. Straßenbelag nach Anspruch 1, **dadurch gekennzeichnet, dass** die Korngrößenverteilung des Sandbetts (2) für eine größte Korngröße von 2,0 bis 4,0 mm, insbesondere von ca. 3,0 mm, und für eine kleinste Korngröße von ca. 0,05 bis 0,10 mm, insbesondere von ca. 0,07 bis 0,01 mm wie folgt ist:
ca. 0 bis 5% der Körner sind kleiner als 0,10 mm
ca. 0 bis 15% der Körner sind kleiner als 0,15 mm
ca. 5 bis 30% der Körner sind kleiner als 0,30 mm
ca. 30 bis 55% der Körner sind kleiner als 0,50 mm
ca. 55 bis 80% der Körner sind kleiner als 1,00 mm
ca. 80 bis 95% der Körner sind kleiner als 2,00 mm
ca. 95 bis 100% der Körner sind kleiner als 3,00 mm
ca. 100% der Körner sind kleiner als 4,00 mm.

3. Straßenbelag nach einem der Ansprüche 1 oder 2, **dadurch gekennzeichnet, dass** die Pflastersteine (3) so auf dem Sandbett (2) verlegt sind, dass sie durch Spalten (4) getrennt sind und durch Sand voneinander beabstandet gehalten werden, der von unten in die Spalten (4) aufsteigt.

4. Straßenbelag nach Anspruch 3, **dadurch gekennzeichnet, dass** die Spalten (4) zwischen angrenzenden Pflastersteinen (3) von oben mit Fugensand (5) verfüllt werden, bei dem der Anteil der feinsten Körner mit einer Korngröße von ≤ 0,10 mm ca. zweimal so groß ist wie derjenige des Sandbetts (2).

5. Straßenbelag nach einem der Ansprüche 1 bis 4, **dadurch gekennzeichnet, dass** die Korngröße ungefähr wie folgt zunimmt:
Sandbett:
im Feinkornbereich: linear bis progressiv, im Zwischenbereich: ungefähr linear, im Grobkornbereich: regressiv
Fugensand:
über den ganzen Bereich progressiv zunehmend.

6. Straßenbelag nach einem der Ansprüche 1 bis 5, **dadurch gekennzeichnet, dass** er eine Wasserdurchlässigkeit von höchstens 0,01 bis 6,00%, insbesondere von 0,10 bis 3,50% hat.

7. Straßenbelag nach einem der Ansprüche 1 bis 6, **dadurch gekennzeichnet, dass** der Asphalt für das Sandbett (2) eine Dichte von ca. 1,0 bis 1,06 g/cm³ bei 25°C, einen Paraffinbestandteil von ca. 2,0 bis 2,5 Gew.-%, eine Nadelstichtiefe bei 25°C von ca. 60 bis 200 dmm, eine Duktilität bei 25°C von ca. 90 bis 100 cm und eine Viskosität bei 135°C von ca. 200 bis 250 mm²/s hat.

8. Straßenbelag nach einem der Ansprüche 1 bis 7, **dadurch gekennzeichnet, dass** für das Sandbett (2) Kiesbrechsand mit einer derartigen Korngrößenverteilung verwendet wird, dass der Leerraumanteil in einer trockenverdichteten Probe höchstens ca. 37,0 bis 39,0, insbesondere 38,5 Vol.-% beträgt.

9. Straßenbelag nach einem der Ansprüche 1 bis 8, **dadurch gekennzeichnet, dass** die Bettung (1) unter dem Sandbett (2) aus Abbruchprodukten besteht.

10. Verfahren zum Bau eines Straßenbelags mit Pflastersteinen (3), die auf einen Sandbett (2) verlegt werden, insbesondere eines Straßenbelags nach einem der Ansprüche 1 bis 9, durch die folgenden Schritte **gekennzeichnet**:
a. Aufbau eines über einer Bettung (1) liegenden Sandbetts (2), das Asphalt in einem Anteil von 1,8 bis 2,2 Gew.-% enthält;
b. Verlegen von Pflastersteinen auf dem noch unverdichteten Sandbett, und zwar so, dass Spalten zwischen angrenzenden Pflastersteinen verbleiben;
c. Einrütteln oder Einklopfen der Pflastersteine in das Sandbett, und zwar so, dass der mit Asphalt versetzte Sand in die Spalten zwischen angrenzenden Pflastersteinen hochsteigt, wobei die Verteilung grober und feiner Körner im Sandbett dergestalt ist, dass während des Einrüttelns oder Einklopfens das Sandbett um ca. 10 bis 20%, insbesondere um ca. 15% verdichtet wird.

11. Verfahren nach Anspruch 10, **dadurch gekennzeichnet, dass**, wenn die Pflastersteine in das Sandbett eingerüttelt oder eingeklopft werden, mit Asphalt versetzter Sand in die Spalten zwischen angrenzenden Pflastersteinen bei einer Spaltbreite von ca. 0,2 bis 0,5 cm ca. 0,3 bis 0,6 cm weit hochsteigt.

12. Verfahren nach einem der Ansprüche 10 - 11, **dadurch gekennzeichnet, dass** das Sandbett in einer Dicke von ca. 3,0 bis 5,0 cm verteilt wird.

13. Verfahren nach einem der Ansprüche 10 - 12, **dadurch gekennzeichnet, dass**, nachdem die Pflastersteine im Sandbett fixiert worden sind, die Spalten zwischen angrenzenden Pflastersteinen mit Fugensand, insbesondere mit Asphalt versetztem Fugensand verfüllt werden.

## Revendications

1. Surface de route pour des zones utilisées par le trafic de véhicules, comportant un pavement qui est supporté par une plate-forme (1), et qui comporte des pierres de pavage préfabriquées (3) réalisées en matériaux naturels ou artificiels, en particulier des pierres de pavage en béton, qui sont disposées sur un lit de sable bitumineux (2),
dans laquelle le composant de bitume du lit de sable (2) par rapport au poids total de ce dernier représente entre environ 1,5 % et 2,5 %, en poids, en particulier environ 1,8 % à 2,2 % en poids,
**caractérisée en ce que**:
la répartition des grains grossiers et fins dans le lit de sable (2) est telle que sous l'action d'un vibrateur sur des pierres de pavage (3) disposées sur le lit de sable non compacté d'origine, le sable est compacté d'environ 10 à 20 %, en particulier d'environ 15 %.

2. Surface de route selon la revendication 1, **caractérisée en ce que** la répartition granulométrique du lit de sable (2) pour une granulométrie maximale de 2,0 à 4,0 mm, en particulier d'environ 3,0 mm, et pour une granulométrie minimale d'environ 0,05 à 0,10 mm, en particulier d'environ 0,07 à 0,01 mm, est la suivante :
environ 0 à 5 % des grains sont plus petits que 0,10 mm
environ 0 à 15 % des grains sont plus petits que 0,15 mm
environ 5 à 30 % des grains sont plus petits que 0,30 mm
environ 30 à 55 % des grains sont plus petits que 0,50 mm
environ 55 à 80 % des grains sont plus petits que 1,00 mm
environ 80 à 95 % des grains sont plus petits que 2,00 mm
environ 95 à 100 % des grains sont plus petits que 3,00 mm
environ 100 % des grains sont plus petit que 4,00 mm.

3. Surface de route selon la revendications 1 ou 2, **caractérisée en ce que** les pierres de pavage (3) sur le lit de sable (2) sont disposées de telle manière qu'elles sont séparées par des espaces (4), et sont maintenues éloignées les unes des autres par du sable qui monte dans les espaces (4) à partir du dessous.

4. Surface de route selon la revendication 3, **caractérisée en ce que** les espaces (4) entre des pierres de pavage adjacentes (3) sont remplis à partir de la partie supérieure avec du sable de jointement (5), la proportion des grains les plus fins avec une granulométrie ≤ 0,10 mm étant environ deux fois aussi grande que celle dans le lit de sable (2).

5. Surface de route selon l'une quelconque des revendications 1 à 4, **caractérisée en ce que** la granulométrie augmente approximativement de la manière suivante :
lit de sable :
dans la zone de grains fins : de manière linéaire à progressive, dans la zone intermédiaire : approximativement de manière linéaire, dans la zone de grains grossiers : de manière régressive.
Sable de liaison :
augmentant progressivement sur toute l'étendue.

6. Surface de route selon l'une quelconque des revendications 1 à 5, **caractérisée en ce qu'**elle a une perméabilité à l'eau au maximum comprise entre 0,01 et 6,00 %, en particulier de 0,10 à 3,50 %.

7. Surface de route selon l'une quelconque des revendications 1 à 6, **caractérisée en ce que** le bitume pour le lit de sable (2) a une densité d'environ 1,0 à 1,06 g/cm³ à 25°C, un composant de paraffine d'environ 2,0 à 2,5 % en poids, une pénétration d'aiguille à 25°C d'environ 60 à 200 dmm, une ductilité à 25°C d'environ 90 à 100 cm, et une viscosité à 135°C d'environ 200 à 250 mm²/s.

8. Surface de route selon l'une quelconque des revendications 1 à 7, **caractérisée en ce que** pour le lit de sable (2), un sable broyé est utilisé avec une répartition granulométrique telle que la proportion d'espace vide dans un échantillon compacté à sec est au maximum d'environ 37,0 à 39,0, en particulier d'environ 38,5 % en volume.

9. Surface de route selon l'une quelconque des revendications 1 à 8, **caractérisée en ce que** la plate-forme (1) sous le lit de sable (2) est constituée de produits de démolition.

10. Procédé pour la construction d'une surface de route avec des pierres de pavage (3) disposées sur un lit de sable (2), en particulier une surface de route selon l'une quelconque des revendications 1 à 9, **caractérisé par** les étapes suivantes :
a. l'érection sur une plate-forme (1) d'un lit de sable sus-jacent (2) contenant du bitume dans une proportion de 1,8 % à 2,2 % en poids,
b. la mise en place de pierres de pavage sur le lit de sable pas encore compacté, afin de laisser des espaces entre des pierres de pavage adjacentes,
c. la vibration ou le martelage des pierres de pavage dans le lit de sable de telle manière que le sable rendu bitumineux monte dans les espaces situés entre des pierres de pavage adjacentes, la répartition de grains grossiers et fins dans le lit de sable étant telle que pendant lesdites vibrations ou ledit martelage, le lit de sable est compacté d'environ 10 à 20 %, en particulier d'environ 15 %.

11. Procédé selon la revendication 10, **caractérisé en ce que** lorsque les pierres de pavage sont mises à vibrer ou martelées dans le lit de sable, du sable rendu bitumineux monte dans les espaces entre des pierres de pavage adjacentes sur une distance d'environ 0,3 à 0,6 cm, étant donnée une largeur d'espace d'environ 0,2 à 0,5 cm.

12. Procédé selon l'une quelconque des revendications 10 à 11, **caractérisé en ce que** le lit de sable est répandu en une épaisseur d'environ 3,0 à 5,0 cm.

13. Procédé selon l'une quelconque des revendications 10 à 12, **caractérisé en ce qu'**après que les pierres de pavage soient devenues fixes dans le lit de sable, les espaces entre des pierres de pavage adjacentes sont remplis de sable de jointement, en particulier du sable de jointement rendu bitumineux.
